

S. P. MORRISON & VAN DOLAH MORRISON.

PACKING.

APPLICATION FILED OCT. 25, 1910.

984,836.

Patented Feb. 21, 1911.

Fig. 1.



Fig. 2.



Fig. 3.



WITNESSES:

C. B. Hoerner

J. L. Whiteman

INVENTORS

Septimus P. Morrison <sup>and</sup>  
Van Dolah Morrison  
Dmitrius D. Hoerner  
By J. H. Hoerner, attorneys.

# UNITED STATES PATENT OFFICE.

SEPTIMUS P. MORRISON, OF STUTTGART, ARKANSAS, AND VAN DOLAH MORRISON, OF INDIANAPOLIS, INDIANA.

## PACKING.

984,836.

Specification of Letters Patent. Patented Feb. 21, 1911.

Application filed October 25, 1910. Serial No. 589,003.

*To all whom it may concern:*

Be it known that we, SEPTIMUS P. MORRISON, a citizen of the United States, residing at Stuttgart, in the county of Arkansas and State of Arkansas, and VAN DOLAH MORRISON, a citizen of the United States, residing at Indianapolis, in the county of Marion and State of Indiana, have invented certain new and useful Improvements in Packing, 10 of which the following is a specification.

This invention relates to improvements in packing for pistons, stuffing-boxes, and for all mechanisms wherein an air, water, oil, steam, ammonia, or gas-tight joint is desired 15 around a reciprocating or rotary portion.

The invention belongs to the same class of packing as that patented to Septimus P. Morrison, by United States Patent No. 926,676, issued June 29, 1909, which packing, as experience has demonstrated, is impracticable for piston-rods and other similar shaft-like reciprocating parts which are apt to be sprung or kinked or bent out of straight alinement, requiring the use of a 25 more or less elastic packing substance which is capable of following, that is, of springing out with or of receding before said imperfections in the reciprocating rod. Also, the packing material of said Patent No. 926,676, 30 being compressible and non-elastic, is impracticable for use as a packing for pistons in cylinders the bores of which have become worn, out of round, as so frequently occurs.

The object of this invention is, therefore, 35 to produce a packing which shall have the lubricant-carrying structure; the capacity for compression whereby, by lateral pressure, it may be thickened in dimensions at right angles to said pressure to accurately 40 fill its box or cylinder; and all of the advantages of the invention of said Patent No. 926,676, with additional attributes, chief among which is that of elasticity.

In the accompanying drawings forming 45 a part hereof, Figure 1 is an exterior view of a collection of granules joined together, showing their irregular formation with innumerable cells existing between said granules. Fig. 2 is a highly magnified view in 50 cross-section of a single granule disconnected from the mass, showing throughout its body

the formation of innumerable communicating cells containing the lubricant. Fig. 3 is a fragmentary view in elevation of a portion of a compressed ring formed out of a 55 mass of the granules, this view showing the exposed cells elongated by the operation of compressing the granules, and also showing the shredded asbestos interwoven throughout the mass.

The body of the packing material comprises innumerable small irregular granules, preferably of substantially the same alloy,—copper, antimony, tin, etc.,—of which Babbitt metal is made, said granules being of 65 irregular shape, and ragged, to increase the adhesion thereto of shredded asbestos by which the granules will eventually be separated, the said granules having innumerable cells throughout their structure forming receptacles for a lubricant, preferably 70 graphite. These granules, as stated, will be separated from each other preferably by shredded asbestos, the sufficiently reduced fibers of which adhere readily to the ragged 75 edges of the granules.

The mixing of the granules with asbestos, oil, and graphite, may be carried forth in various ways, that is, one ingredient may be mixed with the mass before the other, but 80 the desirable way of mixing the several parts we have found is substantially as follows: A sufficient number of granules to form a packing ring is first placed in a receptacle; to this mass shredded asbestos is 85 added, which is stirred until the two become thoroughly mixed; a mixture of graphite with oil, wax, or the like, is then applied to the mass after which the mass is heated so that as the air within the cells becomes 90 heated and expands it escapes from the cells, during which process the cells are filled by the inflow of the lubricant. The mass is now in condition to form rings or packings for different purposes. In case it is desired 95 to form a piston ring, the mass is distributed around a piston and when a clamping-ring is placed in position and pressure is applied the mass is compressed and readily shapes itself to conform to the contour of 100 the adjacent walls, thereby making a smooth and tight joint. As before stated, the metal-

lie structure of the granules is compressible but not elastic, and its cellular formation lends itself to such compression. The asbestos, besides being free from any chemical objections and being a poor heat conductor and practically indestructible from heat, possesses a degree of elasticity which gives the required resiliency to the packing-mass of which it is a part. This resiliency causes the packing to yield under pressure of a bent piston rod or the like and to spring back after the bent part of the rod has passed and to close in against a hollow of said rod, thus maintaining a constant tight joint, and with equal facility it provides a tight packing for pistons operating in out-of-round cylinders.

The packing here described has inherent elasticity to a slight degree by reason of the asbestos, which makes the packing more adaptable to superheated steam, and also for gas and gasolene engines wherein a high temperature obtains.

Our above described packing is sufficiently pliable to be used on movable brass rods and valve stems without danger of fluting the brass surfaces of said rods and stems.

We have here mentioned Babbitt metal, asbestos, and graphite, as illustrative materials, and as preferred ones so far as our experience has gone, but other materials may be substituted with good results without departing from the spirit of our invention

and we therefore do not desire to be limited to the ingredients named, but

What we do claim as new and desire to secure by Letters Patent, is—

1. As a new article of manufacture, a unitary cellular poriferous elastic structure, whose cells are charged with a lubricant.

2. As a new article of manufacture a unitary elastic structure comprising a compressible non-elastic cellular poriferous metal-body in granules, an elastic mineral separating said granules, and a lubricant charging the cells of said metal-body.

3. As a new article of manufacture, a unitary elastic structure comprising a compressible non-elastic cellular poriferous metal-body in a plurality of divided granules, said granules having sharp ragged edges, an elastic substance separating said granules and retained by the edges of the latter, and a lubricant charging the cells of said metal-body.

In witness whereof, we have hereunto set our hands and seals.

SEPTIMUS P. MOREISON. [L. S.]  
VAN DOLAH MORRISON. [L. S.]

Witnesses to signature of S. P. Morrison:

N. H. LECOCQ,  
C. E. PETTIT.

Witnesses to signature of V. D. Morrison:

J. A. MINTURN,  
FRANK O. FITTON.